

## UNITED STATES PATENT OFFICE

2,214,431

ALUMINUM - COPPER-NICKEL-MAGNESIUM  
ALLOY CONTAINING IRON AND COLUM-  
BIUM

Alfred John Murphy, Petts Wood, and Stanley  
Alfred Edward Wells, Teddington, England, as-  
signors, by mesne assignments, to Electro Met-  
allurgical Company, New York, N. Y., a corpora-  
tion of West Virginia

No Drawing. Original application April 16, 1937,  
Serial No. 137,280. Divided and this applica-  
tion August 14, 1939, Serial No. 290,073. In  
Great Britain May 5, 1936

## 2 Claims. (Cl. 75—142)

This invention comprises improvements in  
aluminum base alloys and in particular aluminum  
alloys of the classes containing copper, or  
nickel, or copper together with nickel, or copper  
5 with nickel and magnesium, or copper with  
nickel, magnesium, iron and silicon, or nickel  
with magnesium, iron and silicon. This applica-  
tion is a division of our application Serial No.  
137,280, filed April 16, 1937.

10 In the production of cast pieces of aluminum  
base alloys, by which may be understood alloys  
containing more than 70% of aluminum, it is de-  
sirable to secure the finest possible size of grain.  
The grain referred to is the, macrostructure  
15 which is recognizable by the naked eye on smooth  
surfaces or sections of the cast pieces after they  
have been etched in suitable reagents, such as  
an aqueous solution of caustic soda, or hydro-  
fluoric acid.

20 In castings a diminution in grain size improves  
the mechanical properties. The finer the grain  
size characteristic of an aluminum alloy, other  
things being equal, the better its founding prop-  
25 erties in that the tendency to cracking in the  
mold is reduced and the production of sound  
castings is facilitated. In cast pieces intended to  
be forged, pressed, extruded or otherwise worked  
mechanically, a fine grain size is desirable be-  
cause it assists the attainment of good mechan-  
30 ical properties in the subsequent working.

The object of the invention is to produce alu-  
minum alloys having a fine grain, and possessing  
in consequence of this fine grain superior me-  
chanical properties in the cast condition and  
35 also when forged and also after heat-treatment  
of the castings and forgings according to known  
processes.

According to this invention, a relatively small  
40 proportion of columbium, also known sometimes  
as niobium, is added to an aluminum alloy, partic-  
ularly an alloy of one of the classes referred  
to, the alloy thereby acquiring a fine grain,  
which is maintained over a wide range of con-  
45 ditions of melting, casting and working. We  
have found it convenient to make the propor-  
tion of columbium 0.1% to 0.2% of the total  
weight of the alloy. We have observed appre-  
ciable grain refinement with as little as 0.05%  
50 of columbium, and on the other hand we have  
not found it generally necessary or desirable to  
exceed 0.5% of columbium.

We have discovered that these beneficial  
effects are exhibited in the classes of alloy men-  
55 tioned above containing the elements set out

below in the proportions stated by way of ex-  
ample:

|           | Per cent   |
|-----------|------------|
| Copper    | 0.5 to 12  |
| Nickel    | 0.5 to 5   |
| Magnesium | 0.1 to 3   |
| Silicon   | 0.2 to 2.5 |
| Iron      | 0.2 to 2   |
| Columbium | 0.05 to 1  |

The beneficial effect of the columbium is not  
dependent upon the manner in which it is in-  
corporated in the alloy, but a convenient pro-  
cedure is to add it in the form of a "hardener"  
or "mother" alloy or prealloy relatively rich in  
columbium. According to one practical process,  
15 the first stage in the incorporation of the colum-  
bium in the aluminum alloy is the preparation  
of an aluminum alloy relatively rich in colum-  
bium from ferro-columbium and aluminum.  
The ferro-columbium may be in the form of an  
20 alloy containing approximately equal parts of  
iron and columbium with impurities such as  
tantalum, silicon and carbon in small propor-  
tions. In preparing the columbium "hardener"  
25 alloy, aluminum is melted in a crucible and its  
temperature raised to 1100° to 1200° C. A weight  
of ferro-columbium equal to approximately one-  
tenth of the weight of aluminum is stirred into  
the molten aluminum, or is carried in a perforated  
30 container which is moved up and down in the  
aluminum, until the addition is entirely dissolved.  
In this way an alloy containing approximately  
5% columbium, 5% iron, with the balance sub-  
stantially aluminum, is obtained. This is cast  
35 into molds remelted in a crucible, allowed to  
solidify and remelted without unnecessary super-  
heating, in order to eliminate gases which may  
have become absorbed through the heating to  
high temperatures in the initial operation. After  
40 this "presolidification" treatment, the alloy is  
cast into suitable ingot molds.

One practical process for making up an alloy  
using the aluminum "hardener" alloy relatively  
rich in columbium may be described. The final  
45 alloy to be made according to this example has  
the following nominal composition:

|           | Per cent  |
|-----------|-----------|
| Copper    | 2.5       |
| Nickel    | 1.5       |
| Magnesium | 0.8       |
| Silicon   | 1.2       |
| Iron      | 1.2       |
| Columbium | 0.1       |
| Aluminum  | Remainder |

The "hardener" alloys employed are: aluminum-nickel with 20% nickel, aluminum-iron-columbium with 5% iron and 5% columbium, aluminum-iron with 10% iron, aluminum-copper with 5% copper, aluminum-silicon with 20% silicon. Aluminum is melted in a crucible and the calculated quantities of "hardeners" are stirred in successively in the order in which they are mentioned above, care being taken that each addition is dissolved before the next is introduced. The final addition is the magnesium in the form of the pure metal. By this procedure it is not necessary to raise the temperature of the metal above 750° C. at any stage during the manufacture of the alloy, which is advantageous from the point of view of avoiding absorption of gas.

The alloy described is suitable for the manufacture of castings and forgings, and responds effectively to the known processes of heat-treatment applicable to aluminum alloys containing copper, nickel, magnesium, silicon and iron. For example, a large improvement in mechanical properties of forgings of the alloy is obtained by a two-stage heat-treatment in which the parts are first heated for 4 hours at 530° C., then quenched in water, reheated for 16 hours at 165° C. and finally quenched in water again.

A valuable feature of the grain refining action of columbium is that it is effective even when the aluminum alloy is raised to a high temperature before casting. As an illustration of the efficacy

of the grain refining action of columbium, it may be mentioned that, when an alloy of the composition stated above is cast at 800° C. into a dried sand mold to form a cylindrical block 3" high and 3" diameter, the grains visible in the macrostructure after etching have diameters of 0.2 to 1 mm., whereas the same alloy not containing columbium, cast under the same conditions, shows a grain diameter of 2.5 to 5 mm.

As compared with a similar alloy not containing columbium, the alloy described above has the advantage, due to the fine grain structure which columbium confers, that the ductility associated with a certain tensile strength is greater.

In the simple alloys of aluminum with copper, such as that containing 7% copper, the incorporation of columbium in the form of an aluminum-columbium alloy refines the grain and improves the strength and ductility of castings.

We claim:

1. Aluminum base alloy containing 0.5% to 12% copper, 0.5% to 5% nickel, 0.1% to 3% magnesium, iron in a proportion not over 2%, 0.05% to 1% columbium, remainder aluminum.
2. Aluminum base alloy containing 0.5% to 12% copper, 0.5% to 5% nickel, 0.1% to 3% magnesium, iron in a proportion not over 2%, 0.1% to 0.5% columbium, remainder aluminum.

ALFRED JOHN MURPHY.

STANLEY ALFRED EDWARD WELLS.